

Patented Mar. 13, 1923.

1,448,288

## UNITED STATES PATENT OFFICE.

WALTER LOTHAR EDUARD EILENDER, OF REMSCHEID, GERMANY, ASSIGNOR, BY  
MESNE ASSIGNMENTS, TO THE CHEMICAL FOUNDATION, INC., A CORPORATION OF  
DELAWARE.

### HIGH-SPEED STEEL FREE FROM TUNGSTEN.

No Drawing.

Application filed March 6, 1917. Serial No. 152,725.

To all whom it may concern:

Be it known that I, WALTER LOTHAR EDUARD EILENDER, a subject of the German Emperor, and residing at Remscheid, Germany, have invented certain new and useful Improvements in High-Speed Steel Free from Tungsten, of which the following is a specification.

It is known, that highspeed steels comprise chrome tungsten-steels with such a content of carbon, that the necessary and sufficient hardness can be obtained.

The content of chromium varies between 3 to 7 p. c. that of tungsten was gradually increased, so that, at the present time the best qualities contain between 18 and 25 p. c.

It is known, that successful experiments have been made to further increase the cutting capacity by addition of other metals, for instance molybdenum, vanadium and cobalt.

I have for some time experimented for the purpose of producing a high speed steel of highest cutting effect without tungsten.

These experiments have shown that steel of the following composition has a cutting capacity equal, at least, to the best makes of highspeed steel hitherto known:

30 C=0.5—0.8 p. c., Mo=6.0—10.0 p. c., Cr=3.0—6.0 p. c., Va=0.15—2.0 p. c., Mn=0.2—0.4 p. c., Si=0.2—0.4 p. c.

The same experiments, moreover, have proved it to be possible to lower the content of vanadium to 0.15 p. c., if 0.5—3.5 p. c. cobalt is added.

It is known that vanadium improves more or less nearly all alloy-steels. It therefore is obvious, that even low additions down to 0.15 p. c. comparatively improve the above

described tungstenless steel. It is not less evident, that when small quantities of vanadium are used, a small amount of cobalt is required, as that metal shows its effect mainly in conjunction with vanadium.

It has been proposed and is therefore known, to add cobalt to known chromium-tungsten-vanadium-molybdenum highspeed steels. The above described highspeed steel without tungsten is new and unknown up to date. The addition of cobalt to it is therefore also new.

The steel may be produced by melting, in crucibles, bar steel containing the required content of vanadium, and adding thereto the requisite amount of the metals molybdenum and chromium, viz, 6 to 10 per cent molybdenum and 3 to 6 per cent chromium, and after proper fusion the fused metal is poured from the crucible into suitable ingot molds, from which it is obtained in the form of ingots.

.5 to 3.5 of the metal cobalt may be added where the content of vanadium is low, as, for example, .15 per cent.

What I claim and desire to secure by Letters Patent as my invention is:

The herein described steel alloy for highspeed steel of highest cutting capacity, containing besides iron also 0.5—0.8 p. c. 70 C, 6.0—10.0 p. c. Mo, 3.0—6.0 p. c. Cr, 0.2—0.4 p. c. Mn, 0.2—0.4 p. c. Si and 0.15—2 p. c. Va.

In testimony whereof I hereunto affix my signature in the presence of two witnesses. 75

WALTER LOTHAR EDUARD EILENDER.

Witnesses:

HELEN NUFER,  
FRANCES NUFER.